

Feb. 12, 1957

T. A. TAYLOR ET AL

2,781,005

METHOD OF REDUCING VANADIUM CORROSION IN GAS TURBINES

Filed June 27, 1951

3 Sheets-Sheet 1

Fig. 1



Fig. 2



Feb. 12, 1957

T. A. TAYLOR ET AL

2,781,005

METHOD OF REDUCING VANADIUM CORROSION IN GAS TURBINES

Filed June 27, 1951

3 Sheets-Sheet 2



By  
Stevens, Davis, Miller & Kauper  
their Attorneys

Feb. 12, 1957

T. A. TAYLOR ET AL

2,781,005

METHOD OF REDUCING VANADIUM CORROSION IN GAS TURBINES

Filed June 27, 1951

3 Sheets-Sheet 3



1

2,781,005

**METHOD OF REDUCING VANADIUM CORROSION  
IN GAS TURBINES**

Tristram Allan Taylor, Countesthorpe, Leicester, John James Macfarlane, Cove, Farnborough, and Norman Stephenson, Narborough, near Leicester, England, assignors to Power Jets (Research and Development) Limited, London, England, a British company

Application June 27, 1951, Serial No. 233,796

Claims priority, application Great Britain June 28, 1950

16 Claims. (Cl. 110—1)

This invention relates to fuel oils containing vanadium and to the treatment and combustion of such oils.

It is desirable from an economic point of view to use natural and low grade residual fuel oils in internal combustion power plant, but it is found that such fuels produce an ash which, if it comes in contact with metals at elevated temperatures, of the order of 650° C. and above, causes a greatly increased rate of corrosion, due at least in part to oxidation of the metal. This occurs even in the case of metals and alloys which in normal circumstances would be resistant to heat at such temperatures. It would appear that there are few, if any, metals or alloys which are able to resist corrosion under these circumstances for any substantial length of time. This oxidation both weakens the metal by reduction of its cross-section and also reduces its creep and fatigue resistance. It is also found that ceramic and refractory substances are similarly attacked.

It is found that the accelerated oxidation is mainly due to the vanadium content of the oil. Low grade residual fuel oils nearly always contain a quantity of vanadium in the form of complex vanadium compounds which, on combustion decompose to yield vanadium pentoxide. It is believed that the accelerated corrosion is due to the fact that the vanadium pentoxide exercises a fluxing action on the protective oxide films of parts exposed to the combustion gases. In this way the film on the surface of the parts exposed is destroyed so that further oxidation can take place. This effect is accelerated at high temperatures of the order of 650° C. and above, since the ash and its vanadium pentoxide content is in a liquid or semi-liquid state and is thus able to come into intimate contact with the protective film. The problem is thus particularly acute in gas turbine plant since turbine inlet temperatures in excess of 600° C. and the use of low grade fuel oil are both desirable from the point of view of economy. In particular the blades are subject to high stresses and hence it is highly desirable to provide some means of protection for them. It is found that turbine blades made of iron-base alloys are particularly liable to attack.

According to the invention, the corrosion of parts in high temperature plant due to the vanadium content of fuel oils being burnt therein is reduced by the addition of an additive with which the vanadium will react in preference to the material of said parts.

Preferably the additive is selected from the group consisting of:

- (a) Magnesium and zinc.
- (b) Oxides of such metals.
- (c) Compounds of such metals yielding the oxide at combustion temperatures.

In the preferred form of the invention, the additive is introduced into the fuel before use. Alternatively it can be added separately immediately prior to or during com-

2

bustion, or even subsequent to combustion, but upstream of the parts exposed to corrosion.

It is believed that in the resulting reaction, the vanadium pentoxide content of the oil tends to combine with the additive to form a stable vanadate in preference to attacking the oxide film of the parts exposed to corrosion. Moreover the resultant ash is normally of a dry friable nature and does not tend to adhere to such parts.

The effective part of the additive appears in each case to be the oxide. Thus if a metal is added to the oil, complex compounds are formed which break down at combustion temperatures to yield the oxide. If the metal itself is added during combustion it will immediately burn to form the oxide. Alternatively in either case a suitable metallic compound which will yield the oxide at combustion temperatures may be used.

The invention will now be more fully described with reference to specific examples and to the accompanying drawings of which:

20 Figure 1 shows a test apparatus in which conditions in a gas turbine plant can be simulated.

Figure 2 shows curves obtained in a test carried out in the apparatus of Figure 1.

Figure 3 shows a gas turbine plant using residual fuel oil.

Figure 4 is a detail of the arrangement of Figure 3.

The efficiency of various additives in neutralising the corrosive effect of vanadium on various alloys can be assessed by laboratory tests now described. The additive and vanadium pentoxide, both in the form of a fine powder are roasted together and mixed with a suitable binder, such as Canada balsam, to form a smooth paste. The paste is then spread over the surface of a test specimen which consists of a cylindrical rod of the alloy in question. The binder is burnt off and the specimen is maintained at high temperature in a furnace for a suitable period of time. The specimen can then be weighed and analysed to ascertain the extent and nature of the corrosion.

*Example 1*

Pastes of various compositions were applied to specimens of a heat resisting nickel-base alloy having the following composition.

|           | Percent |
|-----------|---------|
| Nickel    | 76.28   |
| Chromium  | 20.10   |
| Titanium  | 2.14    |
| Aluminium | 0.37    |
| Silicon   | 0.42    |
| Iron      | 0.31    |
| Manganese | 0.18    |
| Carbon    | 0.10    |

55 The specimens were maintained at a temperature of 700° C. for 100 hours, and the table below shows the amounts of alloy oxide formed in each case. The first column shows the equivalent composition of the paste and the second column shows the weight gain in milligrams due to oxide formation, there being one milligram of vanadium pentoxide in the paste applied per square centimeter of surface of the specimen.

|   |               |           |
|---|---------------|-----------|
| 1 | Uncoated      | 0.5 mgs.  |
| 2 | $V_2O_5$      | 6.7 mgs.  |
| 3 | $3CaO.V_2O_5$ | 0.6 mgs.  |
| 4 | $3ZnO.V_2O_5$ | -0.3 mgs. |
| 5 | $3MgO.V_2O_5$ | 0.4 mgs.  |

70 The comparative amounts of corrosion with no coating of paste and with a coating of vanadium pentoxide only are given for comparison. The figure for zinc is shown as being negative. This is due to the fact that the ash formed tends to flake off the specimen due to its friable

nature. In each case the corrosion is reduced to an extent comparable to the natural corrosion which would take place in the absence of vanadium.

Although from the above series of tests, it would appear that a calcium compound would be the most suitable additive from an economic point of view, it is found in practice that certain difficulties arise in the use of this element. Most residual fuel oils also contain a certain amount of sulphur and there is a tendency for the calcium to react with the sulphur to form calcium sulphate in preference to forming a vanadium compound. Hence calcium will only be suitable for use with sulphur free oils, or in cases where some means of removing the sulphur is used. It is found however that zinc and magnesium are not subject to this disadvantage, probably because their sulphates are unstable at the temperatures concerned.

It will be seen that the composition of the paste in each case corresponds to the orthovanadate of the metal concerned; i. e. a salt having the formula  $M_3(VO_4)_2$  for a divalent element such as zinc or magnesium. If a smaller quantity of the additive is introduced, the rate of corrosion is not greatly reduced, probably because a certain amount of free vanadium pentoxide will still be present in the ash.

A test approximating more closely to the conditions actually existing in a gas turbine plant will now be described with reference to Figure 1 of the accompanying drawings.

The test rig consists essentially of a combustion chamber adapted to burn heavy fuel oil and a test section containing dummy blades of the material to be tested. Compressed air is blown under pressure and preheated if necessary through duct 1 into the primary combustion zone 2 of a combustion chamber 3 of the cyclone or vortex type. This chamber is of the type described in British Patent No. 639,468 and will not therefore be further described here. The combustion gases leave through an axial outlet 4 and then passes through voulte 5 into the rectangular test section 6. Mounted within this section are test pieces 7 which are similar in shape to normal gas turbine blades but are uncambered. The combustion gases are then discharged to atmosphere.

With this apparatus heavy fuel oil of any desired composition can be burnt. After a test of suitable duration, the dummy blades can be removed and weighed and analysed and hence the extent and nature of the corrosion ascertained.

#### Example II

In a series of tests using the above apparatus, a fuel oil having a viscosity of 100° F. or 536 Redwood seconds and the following composition was used.

|          | Percent |
|----------|---------|
| Carbon   | 85.68   |
| Hydrogen | 10.97   |
| Sulphur  | 2.48    |
| Ash      | 0.05    |

The ash comprised the following ingredients:

|                    | Percent |
|--------------------|---------|
| Vanadium pentoxide | 65      |
| Sodium monoxide    | 2.5     |
| Nickel oxide       | 9       |

It was found that this ash began to melt at a temperature of about 650° C.

The dummy blades were of the nickel base heat resisting nickel-base alloy mentioned above.

This fuel was burnt in the apparatus of Figure 1 and the amount of oxidation of the dummy blades ascertained by analysis. The experiment was repeated with zinc naphthenate added to the oil in a quantity giving the equivalent of  $3ZnO \cdot V_2O_5$ . In each case the test duration was 50 hours.

The resulting rates of oxidation are shown in the curves A and B of Figure 2. The ordinate represents the alloy

oxide formed in mgs./sq. cm./hr. and the abscissa the blade temperature in degrees C. The upper curve A represents the combustion of fuel without the additive and the lower curve B with the additive. It will be seen for example that at 750° C., the corresponding rates of oxidation are respectively 0.1755 and 0.0125. The additive thus reduces the corrosion to about 7% of its normal value, and it is believed that this approximates to the rate of corrosion which would occur even if no vanadium were present.

Other organic compounds such as the corresponding oleate, stearate, or linoleate could be used, all being soluble in oil. From an economic point of view it would be preferable to add the oxide, hydroxide or carbonate dissolved or suspended in oil, water or other liquid medium. In some cases it is possible to add the powdered metal itself, since for example, certain residual oils will attack zinc directly to form complex organic compounds.

Magnesium can be added in the same way.

As stated above the additive may alternatively be directly introduced into the combustion chamber or into the vicinity of the parts exposed to corrosion. This application of the invention is illustrated with reference to Figures 3 and 4 of the drawings. The compressor and turbine in Figure 3 are shown partly in section.

Figure 3 shows diagrammatically a gas turbine plant suitable for burning residual fuel oil. Air enters through duct 11 as indicated by arrow A and then passes into the axial flow multistage compressor 12. The compressor rotor 13 is mounted in bearing 14 and is connected by shaft 15 to the turbine rotor 16. The compressed air passes from the compressor 12 through ducting 17, 18 and 19 into a cyclone or vortex type combustion chamber 20, which will be more fully described below. The combustion gases then pass through an annular duct 21 to the turbine 22 and are discharged through exhaust duct 23.

The combustion chamber 20 is generally of the type described in said British Patent No. 639,468, and comprises a primary flame tube 31, shown in section in Figure 4, leading tangentially into a vortex chamber 32. The air is delivered from the duct 19 as indicated by arrow B, and the flow is then divided by an inner duct 33 supported co-axially within the flame tube by rings of vanes 34 and 35. Part of the air is delivered directly into the combustion zone 36 of the flame tube through the annular space between the duct 33 and the wall of the flame tube, while the remainder passes through the interior of the duct 33. Mounted within this duct is a perforated substantially frusto-conical flame stabilizing baffle 37. Part of the remainder of the air passes through swirl vanes 38 at the upstream end of the baffle 37 while the rest passes through the holes in the baffle.

Since heavy residual oil is to be used, it is desirable to inject the fuel by means of an air blast burner 39, by which is meant a burner in which atomisation of the fuel is effected by means of a blast of compressed air. Fuel and compressed air are respectively supplied to the burner through pipes 40 and 41.

As explained above there is a tendency for the turbine rotor and stator blades 24 and 25 to be corroded by the vanadium content of the fuel. To reduce this corrosion, a suitable additive is introduced into the air blast through branch pipe 42 from a tank 43, the quantity introduced being determined by valve 44. The additive is thus entrained in the air and mixes with the fuel in the combustion chamber to neutralise the vanadium as explained previously. Similar additives may be used to those which are mixed directly with the oil prior to combustion.

The introduction of additive into the oil before use is also shown in Figure 4. The tank 43 containing the additive is connected to the fuel tank 45 by a pipe 46. After the fuel tank 45 is filled, a suitable quantity of the additive is allowed to run in from tank 43 by opening valve 47. In this case it will be unnecessary to introduce additive into the air blast.

We claim:

1. In a gas turbine plant in which fuel oil containing vanadium and sulphur is burnt and which includes heat-resistant metallic parts exposed to the resultant stream of hot combustion gases at a temperature in excess of 650° C. and normally liable to be corroded by the vanadium pentoxide content of the ash resulting from the combustion of said oil, the method of reducing said corrosion comprising the step of introducing into the plant upstream of said parts an additive selected from the group consisting of magnesium and zinc oxides and magnesium and zinc compounds yielding the oxide at the temperature of said hot combustion gases, the quantity of additive introduced being such that the molecular ratio of the minimum oxide content thereof to the vanadium pentoxide content of the ash is 3 to 1.
2. In a gas turbine plant in which fuel oil containing vanadium and sulphur is burnt and which includes heat-resistant metallic parts exposed to the resultant stream of hot combustion gases at a temperature in excess of 650° C. and normally liable to be corroded by the vanadium pentoxide content of the ash resulting from the combustion of said oil, the method of reducing said corrosion comprising the step of introducing into the plant upstream of said parts an additive selected from the group consisting of magnesium and zinc, the minimum quantity of oxide introduced being related to the quantity of vanadium pentoxide in the ash in the molecular ratio 3 to 1.
3. In a gas turbine plant in which fuel oil containing vanadium and sulphur is burnt and which includes heat-resistant metallic parts exposed to the resultant stream of hot combustion gases at a temperature in excess of 650° C. and normally liable to be corroded by the vanadium pentoxide content of the ash resulting from the combustion of said oil, the method of reducing said corrosion comprising the step of introducing into the plant upstream of said parts an additive selected from the group consisting of zinc oxide and zinc compounds yielding the oxide at the temperature of said hot combustion gases, the quantity of said additive introduced being such that the molecular ratio of the minimum zinc oxide content thereof to the vanadium pentoxide content of the ash is 3 to 1.
4. In a gas turbine plant in which fuel oil containing vanadium and sulphur is burnt and which includes heat-resistant metallic parts exposed to the resultant stream of hot combustion gases at a temperature in excess of 650° C. and normally liable to be corroded by the vanadium pentoxide content of the ash resulting from the combustion of said oil, the method of reducing said corrosion comprising the step of introducing zinc oxide into the plant upstream of said parts, the minimum quantity of zinc oxide introduced being related to the quantity of vanadium pentoxide in the ash in the molecular ratio 3 to 1.
5. A residual fuel oil containing sulphur and a small quantity of vanadium in the form of naturally occurring vanadium compounds which give rise to the presence of a quantity of vanadium pentoxide,  $V_2O_5$ , in the ash resulting from the combustion of said oil, which ash is normally liable to cause corrosion of heat-resistant metallic parts exposed to the combustion products of the oil at temperatures in excess of 650° C. and further containing a quantity of the oxide of a metal M selected from the group consisting of magnesium and zinc, whereby said corrosion is reduced, the minimum quantity of the oxide,  $MO$ , and the quantity of the vanadium pentoxide in the ash being related in the proportion  $3MO:V_2O_5$ .
6. A residual fuel oil containing sulphur and a small quantity of vanadium in the form of naturally occurring vanadium compounds which give rise to the presence of a quantity of vanadium pentoxide,  $V_2O_5$ , in the ash resulting from the combustion of said oil, which ash is normally liable to cause corrosion of heat-resistant metal-
- lic parts exposed to the combustion products of the oil at temperatures in excess of 650° C. and further containing a quantity of zinc oxide whereby said corrosion is reduced, the proportion of the minimum quantity of zinc oxide to the quantity of vanadium pentoxide in the ash being  $3ZnO:V_2O_5$ .
7. A residual fuel oil containing sulphur and a small quantity of vanadium in the form of naturally occurring vanadium compounds which give rise to the presence of a quantity of vanadium pentoxide,  $V_2O_5$ , in the ash resulting from the combustion of said oil, which ash is normally liable to cause corrosion of heat-resistant metallic parts exposed to the combustion products of the oil at temperatures in excess of 650° C. and further containing a quantity of magnesium oxide whereby said corrosion is reduced, the proportion of the minimum quantity of magnesium oxide to the quantity of vanadium pentoxide in the ash being  $3MgO:V_2O_5$ .
8. A fuel oil containing sulphur and a small quantity of vanadium in the form of naturally occurring vanadium compounds which give rise to the presence of a quantity of vanadium pentoxide in the ash resulting from the combustion of said oil, which ash is normally liable to cause corrosion of heat-resistant metallic parts exposed to the combustion products of the oil at temperatures in excess of 650° C. and further containing a quantity of a compound yielding at temperatures in excess of 650° C. the oxide of a metal selected from the group consisting of magnesium and zinc whereby said corrosion is reduced, the molecular ratio of the oxide content of the compound to the quantity of vanadium pentoxide in the ash being at least 3 to 1.
9. In a gas turbine plant in which fuel oil containing vanadium and sulphur is burnt and which includes heat resisting metal parts exposed to the resultant stream of hot combustion gases at a temperature in excess of 650° C. and normally liable to be corroded by the vanadium pentoxide content of the ash resulting from combustion of said oil, the method of reducing said corrosion comprising the step of introducing into the plant upstream of said parts a compound yielding at temperatures in excess of 650° C. the oxide of a metal selected from the group consisting of magnesium and zinc, the quantity of said compound introduced being such that the molecular ratio of the minimum oxide content thereof to the vanadium pentoxide content of the ash is 3 to 1.
10. A method as claimed in claim 9 wherein said compound is an oil-soluble organic compound of a metal selected from the group consisting of magnesium and zinc.
11. In a gas turbine plant in which fuel oil containing vanadium and sulphur is burnt and which includes heat resisting metal parts exposed to the resultant stream of hot combustion gases at a temperature in excess of 650° C. and normally liable to be corroded by the vanadium pentoxide content of the ash resulting from the combustion of said oil, the method of reducing said corrosion comprising the step of introducing into the plant upstream of said parts a magnesium compound yielding magnesium oxide at temperatures in excess of 650° C., the quantity of said compound introduced being such that the molecular ratio of the minimum magnesium oxide content thereof to the vanadium pentoxide content of the ash is 3 to 1.
12. In a gas turbine plant in which fuel oil containing vanadium and sulphur is burnt and which includes heat resisting metal parts exposed to the resultant stream of hot combustion gases at a temperature in excess of 650° C. and normally liable to be corroded by the vanadium pentoxide content of the ash resulting from the combustion of said oil, the method of reducing said corrosion comprising the step of introducing into the plant upstream of said parts a zinc compound yielding zinc oxide at temperatures in excess of 650° C., the quantity of said compound introduced being such that the molecular ratio of the minimum zinc oxide content thereof to the vanadium pentoxide content of the ash is 3 to 1.

13. In a gas turbine plant in which fuel oil containing vanadium and sulphur is burnt and which includes heat resisting metal parts exposed to the resultant stream of hot combustion gases at a temperature in excess of 650° C. and normally liable to be corroded by the vanadium pentoxide of the ash resulting from the combustion of said oil, the method of reducing said corrosion comprising the step of introducing into the plant upstream of said parts an additive selected from the group consisting of magnesium oxide and magnesium compounds yielding the oxide at the temperature of said hot combustion gases, the quantity of said additive introduced being such that the molecular ratio of the minimum magnesium oxide content thereof to the vanadium pentoxide content of the ash is 3 to 1.

14. In a gas turbine plant in which fuel oil containing vanadium and sulphur is burnt and which includes heat resisting metal parts exposed to the resultant stream of hot combustion gases at a temperature in excess of 650° C. and normally liable to be corroded by the vanadium pentoxide content of the ash resulting from the combustion of said oil, the method of reducing said corrosion comprising the step of introducing magnesium oxide into the plant upstream of said parts, the minimum quantity of magnesium oxide introduced being related to the quantity of vanadium pentoxide in the ash in the molecular ratio 3 to 1.

15. A residual fuel oil containing sulphur and a small quantity of vanadium in the form of naturally occurring vanadium compounds which give rise to the presence of a quantity of vanadium pentoxide in the ash resulting from the combustion of said oil, which ash is normally liable to cause corrosion of heat-resisting metallic parts exposed to the combustion products of the oil at temperatures in excess of 650° C., and further containing a quantity of a zinc compound yielding zinc oxide at tem-

peratures in excess of 650° C. whereby said corrosion is reduced, the molecular ratio of the zinc oxide content of the compound to the quantity of vanadium pentoxide in the ash being at least 3 to 1.

5 16. A residual fuel oil containing sulphur and a small quantity of vanadium in the form of naturally occurring vanadium compounds which give rise to the presence of a quantity of vanadium pentoxide in the ash resulting from the combustion of said oil, which ash is normally liable 10 to cause corrosion of heat resisting metallic parts exposed to the combustion products of the oil at temperatures in excess of 650° C., and further containing a quantity of a magnesium compound yielding magnesium oxide at temperatures in excess of 650° C. whereby said corrosion 15 is reduced, the molecular ratio of the magnesium oxide content of the compound to the quantity of vanadium pentoxide in the ash being at least 3 to 1.

#### References Cited in the file of this patent

##### UNITED STATES PATENTS

|           |                 |               |
|-----------|-----------------|---------------|
| 1,350,268 | Skinner         | Aug. 17, 1920 |
| 1,666,523 | Bailey          | Apr. 17, 1928 |
| 2,401,285 | Woodward et al. | May 28, 1946  |
| 2,552,851 | Gist            | May 15, 1951  |
| 2,579,614 | Ray             | Dec. 25, 1951 |

##### FOREIGN PATENTS

|         |               |               |
|---------|---------------|---------------|
| 445,506 | Great Britain | Apr. 14, 1936 |
| 496,692 | Great Britain | Dec. 5, 1938  |

##### OTHER REFERENCES

"Symposium on Corrosion of Materials at Elevated Temperatures," Special Tech. pub. No. 108 pub. by American Society for Testing Materials, presented June 26, 1950, pp. 97-102, 44-68v.